

July 4, 1939.

B. H. DE LONG ET AL

2,165,035

HEAT RESISTING ALLOY STEEL

Filed Aug. 13, 1938

Fig 1



Fig 2



Fig 3



Fig 4



BY *W. H. De Long* INVENTORS  
and *Oscar V. George*

ATTORNEYS  
*W. H. De Long*

## UNITED STATES PATENT OFFICE

2,165,035

## HEAT RESISTING ALLOY STEEL

Berton H. De Long and Omar V. Greene, near  
Reading, Pa., assignors to The Carpenter Steel  
Company, Reading, Pa., a corporation of New  
Jersey

Application August 13, 1938, Serial No. 224,702

2 Claims. (Cl. 75—126)

Our invention relates to alloy steels which are characterized by heat resisting qualities at high temperatures, the main object being to provide an improved alloy which will advantageously combine non-scaling quality, unusual strength, and resistance to abrasion at such temperatures; and it consists essentially in employing the known alloy elements carbon, manganese, silicon and chromium in scientifically determined critical proportions which insure the securing of the predetermined desired qualities, as fully set forth in the following specification taken in connection with the accompanying drawing and specifically defined in the subjoined claims.

15 In the drawing, which indicates graph charts of steel embodying our invention, with one element varying in quantity.

Fig. 1 indicates a carbon variance.

Fig. 2 indicates a manganese variance.

20 Fig. 3 indicates a silicon variance, and  
Fig. 4 indicates a chromium variance.

That added scale resistance is imparted to steel by the use of chromium and silicon, singly or jointly, is well-known in the art, but to the best 25 of our knowledge, the beneficial effect of manganese in this respect has not heretofore been recognized. We are further aware that manganese and silicon or manganese, silicon and chromium have been added to steel in various 30 proportions for other useful purposes, but never in the critical proportions which insure predicted desirable results as provided for by our present invention, the type analysis of which is as follows:

|                                 | Percent |
|---------------------------------|---------|
| Carbon—approximately            | .40     |
| Manganese—approximately         | 8       |
| Silicon—approximately           | 4.50    |
| Chromium—approximately          | 2.75    |
| Balance substantially all iron. |         |

40 Our tests show that this alloy possesses an unpredictably high degree of scale resistance when exposed to incandescent temperatures such as are encountered in furnaces, kilns, internal combustion engines, etc. As a means of demonstrating this high degree of scale resistance, we take machined specimens and expose them continuously in an oxidizing furnace atmosphere at 1600° F. for eight hours and find only a slight 45 discoloration of the surface with negligible change in weight. For convenience, we rate the scale

resistance of various alloys exposed to this test in the following empirical manner.

| Scale resistance rating | Appearance of the surface                                     | 5  |
|-------------------------|---------------------------------------------------------------|----|
| 1                       | Practically no scale—surface bright.                          |    |
| 2                       | Very light powdery free scale—surface bright.                 |    |
| 3                       | Light gray powdery free scale—surface generally bright.       |    |
| 4                       | Gray free scale—surface slightly discolored.                  | 10 |
| 5                       | Light grayish black adhering scale.                           |    |
| 6                       | Heavy black or heavy dark gray free scale—surface discolored. |    |
| 7                       | Heavy gray or black adhering scale.                           |    |

The critical nature of the particular analysis 15 combination set forth may readily be proved by melting a series of alloys in which any three of the essential elements are kept constant and the fourth element is permitted to vary above and below the optimum percentage set forth. 20 Four such series of tests are illustrated in the drawing. Figure 1 illustrates the scale resistance of a series of alloys each of which contains manganese approximately 8%, silicon approximately 4.50%, and chromium approximately 2.75%; and 25 in which the carbon is permitted to vary from practically nothing to over 2%. The carbon variable is plotted horizontally, and the scale resistance number is plotted vertically. It will be seen that scale resistance gradually improves as 30 the carbon is increased, reaches an effective maximum between about .20% and .75%, and then decreases as the carbon is further increased.

Figure 2 shows the scale resistance of a series 35 of alloys each of which contains carbon approximately .40%, silicon approximately 4.50%, and chromium approximately 2.75%; and in which the manganese is permitted to vary from about .40% to about 60%. It will be seen that the scale resistance gradually improves as the manganese 40 is increased, reaches an effective maximum between about 6% and 10%, and then decreases as the manganese is further increased.

Figure 3 shows the scale resistance of a series 45 of alloys each of which contains carbon approximately .40%, manganese approximately 8%, chromium approximately 2.75%, and in which the silicon is permitted to vary from about 2% to about 30%. It will be seen that the scale resistance gradually improves as the silicon is increased, reaches an effective maximum between 50

3.5% and 6.5%, and then decreases as the silicon is further increased.

Figure 4 shows the scale resistance of a series of alloys each of which contains carbon approximately .40%, manganese approximately 8%, silicon approximately 4.50%; and in which the chromium is permitted to vary from substantially nothing to about 30%. It will be seen that the scale resistance gradually improves as the chromium is increased, reaches an effective maximum between 1.5% and 4.5%, and then decreases as the chromium is further increased.

To the best of our knowledge, the critical nature of this particular combination of elements with respect to scale resistance is new and such alloys have never before been made for heat resisting, scale resisting or any other purposes.

Alloys for use at elevated temperatures should not only be highly resistant to scale and surface deterioration, but should, if possible, also possess a high degree of mechanical strength at elevated temperatures. A simple criterion of strength at elevated temperatures is found in the Brinell hardness test. Specimens of the alloys being tested are heated to the desired temperature and are then subjected to the Brinell hardness test. Relatively high Brinell hardness numerals indicate relatively high strength at that temperature. The following table illustrates the comparative scale resistance and red hardness of our new critical alloy combination and certain other ferrous alloys which have been extensively used for heat resisting applications.

find that the desirable scale resisting and red hard properties are usefully retained with such extra alloying elements present, alone or in combination, up to perhaps 3%. Our alloy can of course contain small percentages of phosphorus and sulphur such as are normally encountered in commercial manufacture, or these elements may be deliberately added in larger quantities for free machining purposes. In the subjoined claims, the expression "balance substantially all iron" contemplates extraneous alloys permissibly present in a total quantity of not more than about 3%.

Our new heat resisting alloy can readily be made in the usual steel making equipment by those familiar with the art. Electric melting in induction or arc furnaces is preferred for conservation of the alloys, appropriate charges of melting stock and ferrous alloys being employed. The alloy is readily malleable, and can be hot hammered or hot rolled into useful shapes with standard steel mill equipment. The alloy may be heat treated for hardness, or softened for machining by suitable thermal treatment.

We have measured the scale resistance and red hardness of our new alloy in the cast, rolled, and forged condition and find that it can be employed in any of these forms for heat resisting purposes such as valves in internal combustion engines, high temperature bolts and studs, furnace parts, and the like.

What we claim is:

1. A heat resisting ferrous alloy having scale

| Alloy No. | Analysis |           |         |          |        |          |                  |                               |
|-----------|----------|-----------|---------|----------|--------|----------|------------------|-------------------------------|
|           | Carbon   | Manganese | Silicon | Chromium | Nickel | Tungsten | Scale resistance | At 1,600° F. Brinell hardness |
| SAE: 3140 | .44      | .60       | .23     | .55      | 1.26   | -----    | 7                | 36                            |
| 934       | .40      | .49       | 4.54    | 8.37     | -----  | -----    | 3                | 39                            |
| 847       | .51      | .22       | .23     | 3.45     | -----  | 13.25    | 5                | 87                            |
| 802       | .41      | .40       | 4.07    | 3.19     | -----  | -----    | 6                | 37                            |
| 856       | .40      | 8.40      | 4.35    | -----    | -----  | -----    | 3                | 71                            |
| 908       | .41      | 8.25      | 4.14    | 2.49     | -----  | -----    | 2                | 95                            |

It will be seen that our preferred composition in alloy 908 compares very favorably with the best scale resistance and red hardness of the older alloys, combining these two desirable properties in one alloy. The excellent properties of alloy 856 are also noteworthy as embodying our critical percentages of silicon and manganese without chromium.

We have experimented with the addition of other alloying elements to the optimum carbon, manganese, silicon, chromium combination set forth adding such elements as nickel, tungsten, selenium, molybdenum, vanadium, copper, aluminum and other common alloying elements, and

resisting property and unusual strength and resistance to abrasion at high temperatures, containing carbon about .40%, manganese about 8.00%, silicon about 4.50%, chromium about 2.75%, and the balance substantially all iron.

2. A heat resisting ferrous alloy having scale resisting property and unusual strength and resistance to abrasion at high temperatures, containing carbon between .20% and .75%, manganese between 6.00% and 10.00%, silicon between 3.5% and 6.5%, chromium between 1.5% and 4.5%, the balance substantially all iron.

BERTON H. DE LONG.

OMAR V. GREENE.

60